# EUROPEAN PATENT SPECIFICATION

(11) **EP 0 775 228 B1**
(45) Date of publication and mention of the grant of the patent: **21.02.2001**
(21) Application number: 95927098.4
(22) Date of filing: 08.08.1995
(51) Int. Cl.: D06M 13/268, D06M 13/256, D06P 1/62, D06P 1/651

(54) **PREVENTION OF PHOTOBLEACHING OF WOOL AND/OR OTHER NATURAL FIBRES**
VERHINDERUNG DER PHOTO-BLEICHUNG VON WOLLE UND/ODER ANDERE NATÜRLICHE FASERN
PREVENTION DE LA DECOLORATION PAR LA LUMIERE DE LA LAINE ET/OU D'AUTRES FIBRES NATURELLES

(30) Priority: 08.08.1994 NZ 26419994
(43) Date of publication of application: 28.05.1997
(73) Proprietor: WOOL RESEARCH ORGANISATION OF NEW ZEALAND INCORPORATED, Lincoln 8152 (NZ)
(72) Inventor: INGHAM, Peter, Edward, Christchurch 8002 (NZ); DODDS, Margaret, Millar, Christchurch (NZ)
(74) Representative: Wharton, Peter Robert
(86) International application number: NZ9500070
(87) International publication number: WO9605357

(56) References cited:
- EP-A- 0 112 120
- EP-A- 0 685 589
- FR-A- 2 398 835
- GB-A- 1 230 145
- GB-A- 1 377 218
- GB-A- 2 186 004
- US-A- 3 683 013
- US-A- 3 930 795
- US-A- 4 217 103
- US-A- 4 270 236
- US-A- 4 295 852
- US-A- 5 207 802
- US-A- 5 240 465
- US-A- 5 250 079
- US-A- 5 350 422
- US-A- 5 428 117

## Description

### FIELD OF THE INVENTION

This invention relates to the use of a compound undergoing photo yellowing for cancelling out the photo bleaching which wool and other similar natural fibres undergo when the wool and/or natural fibres are first exposed to sunlight, such as behind glass.

### BACKGROUND OF THE INVENTION

Photobleaching (sometimes called "first fade" or "red fade") is seen as a rapid but limited on-tone fading of the natural creamy yellow of wool.

Yellowness induced from processing eg, dry-heat, hydrothermal or alkali yellowing is also photobleachable.

The bulk of the photobleaching occurs within 5-10 hours of the wool being exposed behind glass to midsummer sunlight and continues at a slower rate for another 40-50 hours.

The colour change caused by photobleaching is a cause of a significant number of consumer complaints particularly in the case of carpets. It is noticeable when furniture is moved revealing a colour difference between the areas of carpet which have been exposed to sunlight and those which have been unexposed.

The primary object of the present invention is to reduce or prevent this initial colour change in wool or wool blend furnishings which occurs on exposure to sunlight thus eliminating consumer complaints due to this cause.

### SUMMARY OF THE INVENTION

According to the present invention there is provided a use of a chemical compound for treating natural fibres for cancelling out the photo bleaching thereof, the chemical compound undergoing photoyellowing at a similar rate to the rate at which the natural fibres undergo photobleaching, the chemical compound being applied in such an amount that the change in yellowness of the treated fibres, when exposed to sunlight, such as behind glass, is reduced or prevented in comparison to untreated fibres.

The preferred class of chemical compounds are known industrially as syntans and may consist of condensation products of aromatic sulphones and/or sulphonic acids.

However other compounds which similarly undergo a photoyellowing at a similar rate to the photobleaching of wool or the like fibres are also suitable. These may include optical brightening agents, tannins, aromatic sulphonic acids etc.

### BRIEF DESCRIPTION OF THE DRAWINGS

Further aspects of the invention will become apparent from the following description, which is given by way of example only and with reference to the accompanying drawings in which:
Figure 1 shows a graph of the change in yellowness of wool felts treated with an aromatic sulphonic acid condensation product over a period of 40 hours exposure to sunlight;
Figure 2 shows a graph of the change in yellowness of whiter wool felts treated with an aromatic sulphonic acid condensation product over a period of 40 hours exposure to sunlight;
Figure 3 shows a graph of the change in yellowness of treated and untreated yarns over a period of 40 hours exposure to sunlight; and
Figure 4 shows a graph of the change in yellowness of treated and untreated yarns over a period of 40 hours exposure to sunlight.

### DESCRIPTION OF THE PREFERRED EXAMPLES

Particular examples of the invention are set out below.

### Example 1

Two scoured loose wool samples of different yellowness were treated with a condensation product of arylsulphonic acids as follows: Wool samples (20g) were treated in a laboratory dyeing apparatus at 75°C with 0, 0.5% and 1% of product on weight of wool (oww).

These samples were rinsed, dried at 60°C then hand carded and packed into a glass ended container at a packing density of 0.10g/cc.

Yellowness values (Y-Z tristimulus values) were measured using a Hunterlab Spectrocolorimeter using a 2° observer and illuminant C before and after exposure to 40 hours midsummer sunlight (Christchurch, NZ).

**Results were:**

| | Initial Y-Z value | Y-Z value after 40 hours sunlight | Δ(Y-Z) |
|---|---|---|---|
| Untreated sample 1 | 5.1 | 0.6 | 4.5 |
| Sample 1 & 0.5% product | 5.7 | 3.6 | 2.1 |
| Sample 1 & 1.0% product | 5.8 | 4.6 | 1.2 |
| Untreated sample 2 | 4.2 | 1.5 | 1.7 |
| Sample 2 & 0.5% product | 4.2 | 3.9 | 0.3 |
| Sample 2 & 1.0% product | 4.4 | 4.2 | 0.2 |

Thus the change in yellowness for the wool samples after 40 hours sunlight exposure was reduced by 73% and 88% respectively.

### Example 2

Two wool felts of different yellowness were treated with 0, 0.25, 0.5, 0.75 and 1% of an aromatic sulphonic acid. The samples were then exposed to midsummer sunlight behind glass and the yellowness measured after 1, 2, 5, 10, 20, and 40 hours using a Hunterlab Spectrocolorimeter as in Example 1.

The results are shown in Figures 1 and 2.

It can be seen in Figures 1 and 2 that wools of different original yellowness require different amounts of chemical to prevent a colour change. Figure 1 shows that increasing amounts of an aromatic sulphonic acid condensation product reduce the extent of photobleaching. At 1 % oww there is a minimal colour change. Results for a whiter wool (Figure 2) show best results are obtained at a treatment rate of 0.5%oww.

### Example 3

The treatment was applied during the dyeing of a commercial production yarn batch of two tonnes. The dyeing was carried out in a longclose single stick hank dyeing machine using Sandolan MF dyes (Sandoz) at 0.8%. As well as the standard auxiliaries 1% hydroylammonium sulphate (HAS) and 0.5% of an aromatic sulphonic acid were added at the beginning of the dyeing. The wool blend had a Y-Z value of 4.6. Samples from this treated batch as well as untreated samples from a previously dyed batch and the untreated, undyed wool were exposed behind 2 mm picture glass to mid-summer sunlight (Christchurch, NZ). Colour measurements were taken prior to exposure and after 1, 2, 5, 10, 20 and 40 hours after exposure using a Hunterlab Spectrocolorimeter. The change in yellowness is recorded as Δ(Y-Z) and this is shown in Figure 3. In Figure 3 it can be seen that after 40 hours exposure to sunlight the treated yarn changed by 0.3 Y-Z units (ie, indiscernible) whereas the untreated yarn changed by 2.3 Y-Z units. (A change in Δ(Y-Z) > 1 is said to be visibly discernible.)

### Example 4

The treatment was applied during commercial loose stock dyeing to a 2.8 tonne batch of wool with an initial Y-Z value of 3.0. Dyeings consisted of 12 lots each of 235 kg dyed with 2:1 premetallised dyes to a light beige shade (0.013% dye). The treatment was applied with other dyeing auxiliaries included 1 % HAS. The level of the aromatic sulphonic acid was 0.4%. The 12 dyeings were blended and processed into yarn which received a scour in a 5 bowl tape scour. This was followed by another 5 bowl chemical setting treatment using 10 g/L of sodium metabisulphite. The yarn was similarly exposed behind 2 mm picture glass to mid-summer sunlight for 40 hours. An untreated control sample and an undyed/untreated wool sample were also exposed. Colour measurements were taken using a Hunterlab Spectrocolorimeter at 0, 1, 2, 5, 10, 20 and 40 hours exposure. The Δ(Y-Z) values (change in yellowness) are shown in Figure 4. Figure 4 shows that after 40 hours exposure the treated yarn has changed by 0.2 Y-Z units and the untreated yarn has changed by 1.5 Y-Z units.

This example shows the treatment is fast to tapescouring and chemical setting if applied during dyeing.

The wool can be treated during scouring, at the dyeing stage or on a continuous carpet processing line. The treatment can be applied to loose wool, wool yarn, wool fabric or carpet.

The level of compound applied depends on the initial yellowness of the wool and the dyestuffs used but can be adjusted so that there is little or no colour change due to photobleaching behind glass.

The addition of 1-2% of hydroxylammonium sulphate (HAS) with the dyeing auxiliaries significantly reduces dyebath yellowing and hence reduces the required amount of syntan compound. For this reason it is recommended that 1-2% HAS be used in conjunction with the syntan compound.

## Claims

1. Use of a compound undergoing photo yellowing for cancelling out the photo bleaching of natural fibres, wherein the compound is undergoing photo yellowing at a similar rate to the rate of photo bleaching of the natural fibres, and the compound being applied in such an amount that the change in yellowness of the treated fibres, when exposed to sunlight, is reduced or prevented in comparison to untreated fibres.

2. Use of a compound as claimed in claim 1 wherein the chemical compound comprises a condensation product of aromatic sulphones.

3. Use of a compound as claimed in claim 1 wherein the chemical compound comprises a condensation product of sulphonic acid.

4. Use of a compound as claimed in claim 1 wherein the chemical compound comprises an optical brightening agent, tanning, or aromatic sulphonic acids.

5. Use of a compound as claimed in any one of the preceding claims wherein the chemical compound is applied during scouring, dyeing or processing of the natural fibres.

6. Use of a compound as claimed in any one of the preceding claims wherein the natural fibre is wool.

7. Use of a compound as claimed in claim 6 wherein the chemical compound is applied to loose wool, wool yarn, wool fabric or carpet.

8. Use of a compound as claimed in any one of the preceding claims wherein the amount of chemical compound applied to the natural fibres depends on the initial yellowness of the wool.

## Patentansprüche

1. Verwendung einer Verbindung, die einem Lichtvergilben unterzogen wird, um das Lichtbleichen von Naturfasern aufzuheben, wobei die Verbindung dem Lichtvergilben mit einer Rate unterzogen wird, die der Rate des Lichtbleichens der Naturfasern ähnlich ist, und wobei die Verbindung in einer solchen Menge angewandt wird, daß die Veränderung der Vergilbung der behandelten Fasern, wenn sie dem Sonnenlicht ausgesetzt sind, im Vergleich zu unbehandelten Fasern verringert oder verhindert wird.

2. Verwendung einer Verbindung nach Anspruch 1,
wobei die chemische Verbindung ein Kondensationsprodukt von aromatischen Sulfonen aufweist.

3. Verwendung einer Verbindung nach Anspruch 1,
wobei die chemische Verbindung ein Kondensationsprodukt von Sulfonsäure aufweist.

4. Verwendung einer Verbindung nach Anspruch 1,
wobei die chemische Verbindung ein optisches Aufhellungsmittel, Tannine oder aromatische Sulfonsäuren aufweist.

5. Verwendung einer Verbindung nach einem der vorhergehenden Ansprüche,
wobei die chemische Verbindung während des Auswaschens, Entfettens, Färbens oder Verarbeitens der Naturfasern angewandt wird.

6. Verwendung einer Verbindung nach einem der vorhergehenden Ansprüche,
wobei die Naturfaser Wolle ist.

7. Verwendung einer Verbindung nach Anspruch 6,
wobei die chemische Verbindung bei loser Wolle, Wollgarn, Wollgewebe oder Teppichen angewandt wird.

8. Verwendung einer Verbindung nach einem der vorhergehenden Ansprüche,
wobei die Menge der bei Naturfasern angewandten chemischen Verbindung von dem anfänglichen Gelbstich der Wolle abhängt.

## Revendications

1. Utilisation d'un composé subissant un photojaunissement, destinée à supprimer le photoblanchiment de fibres naturelles, caractérisée en ce que le composé subit un photojaunissement à un taux similaire au taux de photoblanchiment des fibres naturelles, et le composé est appliqué dans une quantité telle que la modification du jaunissement des fibres traitées, lorsqu'elles sont exposées au soleil, est réduite ou empêchée en comparaison à des fibres non traitées.

2. Utilisation d'un composé selon la revendication 1, caractérisée en ce que le composé chimique comprend un produit de condensation de sulfones aromatiques.

3. Utilisation d'un composé selon la revendication 1, caractérisée en ce que le composé chimique comprend un produit de condensation de l'acide sulfonique.

4. Utilisation d'un composé selon la revendication 1, caractérisée en ce que le composé chimique comprend un azurant, un agent de tannage, ou des acides sulfoniques aromatiques.

5. Utilisation d'un composé selon l'une quelconque des revendications précédentes, caractérisée en ce que le composé chimique est appliqué lors du dessuintage, de la teinture ou du traitement des fibres naturelles.

6. Utilisation d'un composé selon l'une quelconque des revendications précédentes, caractérisée en ce que la fibre naturelle est la laine.

7. Utilisation d'un composé selon la revendication 6, caractérisée en ce que le composé chimique est appliqué à de la laine en vrac, du fil de laine, un tissu ou un tapis de laine.

8. Utilisation d'un composé selon l'une quelconque des revendications précédentes, caractérisée en ce que la quantité de composé chimique appliquée sur les fibres naturelles dépend du jaunissement initial de la laine.
